

# UNITED STATES PATENT OFFICE.

FREDERICK W. DUNNELL, OF SPRINGFIELD, MASSACHUSETTS, ASSIGNOR,  
BY DIRECT AND MESNE ASSIGNMENTS, OF ONE-SEVENTH TO P. A.  
DONOGHUE, ONE-SEVENTH TO JAMES J. MURPHY, ONE-SEVENTH TO  
JAMES H. EDMONDS, ONE-SEVENTH TO HENRY M. FREYER, ONE-SEVENTH  
TO DONALD B. RICE, AND ONE-SEVENTH TO CLIFFORD B. POTTER, ALL  
OF SPRINGFIELD, MASSACHUSETTS.

## COMPOSITE BLOCK AND PROCESS OF MAKING SAME.

No. 823,038.

Specification of Letters Patent.

Patented June 12, 1906.

Application filed September 24, 1902. Renewed February 17, 1906. Serial No. 301,631.

*To all whom it may concern:*

Be it known that I, FREDERICK W. DUNNELL, a citizen of the United States, and a resident of Springfield, Hampden county, 5 Massachusetts, have invented certain new and useful Improvements in Composite Blocks and Processes of Making the Same, of which the following is a specification.

My invention has relation to a new product or composition of matter for use for paving-blocks, railroad-ties, and other analogous purposes.

The product consists, essentially, in a block formed of disintegrated scraps of leather treated chemically and reduced to a composite mass or block.

The process consists in a method of treatment hereinafter set forth and claimed.

It is my object to produce a block of any 20 desired shape which shall possess in the highest attainable degree the properties of durability, imperviousness to moisture, strength, and solidity. To this end I make use of leather scraps or refuse leather of any kind, 25 which I treat as follows: The scraps or pieces of leather are first ground up or comminuted by grinding or attrition. I prefer to subject the leather to a grinding or rubbing process rather than cutting or chopping it up, since 30 the disintegrating it by attrition is better calculated to preserve the continuity of the fabric and can be readily accomplished by the use of a grindstone, such as are used in the manufacture of wood-pulp or paper. The 35 ground or comminuted mass of leather is then introduced into a tub or vat provided with a suitable quantity of water to saturate or thoroughly moisten the shredded leather. The water may be worked through the mass of 40 scrap leather by means of a beater or wheel, and after this step I add a quantity of coal-tar pitch, rock-asphalt, or other similar material, which should be thoroughly worked into and through the mass of moistened 45 leather. This serves as a binder or cement to cement together the mass when it is dried and, furthermore, renders the product quite impervious to moisture. Without such a moisture-proof cement or binder the composite leather blocks would soak up moisture 50 when exposed to the weather, swell up, and spoil. I may also add with good results a small quantity of linseed-oil or some mineral oil and a little resin.

The proportions of the respective ingredients used do not require to be exact, but I have attained excellent results by using the several ingredients in the following proportions: Mix up, say, eighty pounds of scrap leather with about fifty gallons of water. 55 After the water has been worked into the leather then add about fifteen gallons of coal-tar pitch, rock-asphalt, or the like and mix this thoroughly with the saturated mass of leather. Instead of using so much coal-tar 60 pitch I may and indeed have used a mixture of ten gallons of coal-tar pitch, five gallons of linseed-oil or mineral oil, and three gallons of melted resin. These three ingredients may be poured into the mass in any order and 65 mixed up together with it. After the ingredients have been thoroughly mixed or worked into the mass the resulting pulp is then run into molds and allowed to dry. This drying 70 process may, if desired, be hastened by the application of pressure, which squeezes out a 75 part of the moisture. When the mass has dried in the mold, it will be found to be a solid homogeneous dark-brown substance impervious to moisture, having great resisting 80 strength and durability. It may be cut up into blocks of any desired shape to suit the different purposes for which it is desired to use it.

It will be understood that the quantities 85 named herein are not at all absolute and that equivalent substances capable of forming the same office in the composition may be employed. For example, if a less quantity of water be used, while the pulp will be less thin 90 and fluid it would probably dry out faster in the mold. The oil is an important ingredient, since by thoroughly permeating the mass of the composition it prevents the percolation of water and consequent deterioration or 95 rotting of the material. It will be understood that I do not confine myself to any predetermined order or mode of mixing the several ingredients, the main point being to secure a thorough and intimate mixing of the 100

various substances before the pulp is run into the mold.

Without attempting to set forth all the various substitutes that may be employed for the ingredients mentioned or the variations which may be made in the practice of my process, what I claim is—

1. The herein-described process of forming a composite block which consists in mixing into a homogeneous pulp, leather shavings, water, coal tar pitch, resin and oil, and thereafter subjecting said pulp to pressure to expel superfluous water and to harden it into a solid mass, substantially as described.
2. A composite block consisting of pulp made of shredded leather saturated with

water and thoroughly mixed with coal-tar pitch, resin and oil, substantially as indicated.

3. The above-described substance comprising a homogeneous mass of shredded leather intimately mixed throughout with water, coal-tar pitch and oil, solidified and hardened under pressure, substantially as described.

In witness whereof I have hereunto set my hand this 18th day of September, 1902.

FREDERICK W. DUNNELL.

In presence of—

ALEX. H. YOUNG,  
C. L. YOUNG.